

March 28, 1939.

V. F. ZAHODIAKIN

2,152,128

METHOD OF MAKING PISTON RINGS

Filed March 13, 1936



INVENTOR  
Victor F. Zahodiakin  
Wood & Wood  
ATTORNEYS

## UNITED STATES PATENT OFFICE

2,152,128

## METHOD OF MAKING PISTON RINGS

Victor F. Zahodiakin, New York, N. Y.

Application March 13, 1936, Serial No. 68,748

3 Claims. (Cl. 29—156.6)

This invention relates to piston rings and the method of manufacturing piston rings, particularly piston rings of the type disclosed in the patent granted to Victor F. Zahodiakin No. 1,957,927 on May 8, 1934. The ring disclosed in the mentioned patent is formed from a strip of metal to provide a series of radially disposed passageways opening at the inner and outer periphery of the ring. In connection with the method herein concerned, reference may also be made to the pending application of Victor F. Zahodiakin filed April 10, 1934, Serial No. 719,885, in which application, the ring is formed by means of series of dies.

It is an object of this invention to provide an improved piston ring and method of forming the same, particularly a ring in which the corrugations forming the oil passageways have sharp corners, the invention including for this purpose an improved die action and preferably a special metal strip stock from which the rings are formed.

It has been discovered herein that swaging changes the physical properties of the material. In the development of the present invention it has been found that a machine forming the strip metal by means of dies has the effect of hardening the metal and that rings thus produced may be made from low carbon steel which after the forming operations produces a tough, strong, and properly hardened ring, having good wearing qualities.

Accordingly it is an object of the present invention to provide a method of making piston rings wherein the strip of metal from which the ring is formed may be of low carbon content, the method bringing about the production of a piston ring having the requisite hardness and toughness for the intended use, this result being achieved by the die action on the metal.

It has also been found that different grades of steel must be used as the speed of production of the machine varies. This is particularly true in connection with the present die arrangement in view of the fact that a series of dies are employed, and it is necessary that these dies have working clearances therebetween for permitting expansion of the parts and for lubricating purposes. If a steel of low carbon content is used, and the machine is operated at high speed, some of the metal will be forced into the clearances between the dies during swaging, creating fins at the corners of the formed strip.

Accordingly it is a further object of the present invention to provide a method of manufacturing piston rings from strip metal, wherein a steel of

low carbon content is delivered to the machine when it is operating at low speed, and a steel of high carbon content is delivered to the machine when it is operating at high speed.

Other objects and certain advantages will be more fully apparent from the drawing, in which:

Figures 1 to 11 inclusive are similar fragmentary views of the piston ring forming machine showing the strip of metal progressing through the machine, and illustrating the various stages of its formation.

Referring to the drawing in detail, it is pointed out that the views are substantial duplicates with the exception of the position of the strip of metal and the positions of the dies. The dies operate generally within a die chamber 15, defined by the walls 16. The strip of metal 17 is delivered or fed through the die chamber through aligned transverse openings 18, which openings are provided through a transversely disposed die guide 19.

The strip of metal passes between sets of dies. These dies are operated and timed by any appropriate mechanism such as cams and levers. For the purpose of identifying the dies throughout the views they have been marked by the numerals 1 to 9 inclusive. The upper set consists of dies 1 to 4 inclusive, and the lower set 5 to 9 inclusive. As will be apparent from an inspection of the views, the respective dies slide upon each other. In order that they may slide in an efficient manner, it is necessary that working clearances be provided, which clearances receive the lubricating oil and permit expansion of the dies and associated parts.

A series of views have been disclosed in order that the multiplicity of die actions may be fully realized, and for the purpose of illustrating the formation of the corrugations and the swaging action for producing square or sharp corners. In the views, arrows have been used to illustrate or indicate which die has moved and the direction of movement thereof.

In Figure 1, the dies are in their initial position prior to the start of the forming operations. In this view, the strip of metal has been advanced to a position where it rests on die 8 with its forward edge coinciding with the edge of die 8.

In the next view, Figure 2, upper die 4 has moved down into engagement with the strip whereby the end of the strip is clamped between dies 4 and 8. Also dies 1, 2, and 3 have moved down very slightly and die 6 has moved the same amount upwardly. Die 3 is then in the proper position for coaction with die 7.

35

40

45

50

55

In Figure 3, dies 7 and 9 have moved upwardly and die 7 has formed one side of a corrugation by coacting with dies 3 and 4. The purpose of moving die 9, which is a pilot die, will be described later since die 9 functions after the strip has progressed further.

In Figure 4, die 2 has moved down completing the corrugation around die 7 by coaction with dies 6 and 7. The corrugation referred to is identified at 20. In Figure 5, die 5 has moved upwardly for the purpose of forming a portion 21 of the next corrugation.

In Figure 6, dies 2 and 7 have been retracted a slight amount. Dies 1, 5, and 8 remain stationary for the purpose of holding the formed strip rigidly in position so that during the swaging action, which is to ensue, there is no chance for the strip to become displaced. The vertical walls 22 of the corrugations cannot be displaced since they are contained between the dies 5, 2, 7, and 4. These walls 22, during the swaging action, are confined so rigidly between the dies as to preclude any change in their original dimension or form. The dies may then be referred to as forming a die box within which the swaging can take place.

The spaces or chambers provided by retraction of dies 2 and 7 are of sufficient size or will contain an amount of metal equal to that which will be swaged into the corners as dies 3 and 6 move against the metal as shown in Figure 7. Dies 3 and 5 have sharp corners and after they force the metal of the crowns of the corrugation toward dies 7 and 2 respectively, the metal flows or is displaced so as to fill up the corners and create sharp edges.

In Figure 8, the dies 1, 2, 4, 5, 7, and 9 are retracted so as to clear the corrugations of the ring for subsequent advance or feed of the strip. In Figure 9 the swaging dies 3 and 6 are retracted leaving the strip entirely free for feed. As indicated in Figure 10, the strip is then fed forwardly against clamping die 4 for the next cycle of operation.

It will be noted that Figure 11 as far as the position of the dies is concerned, is a duplicate of Figure 2. However, the strip has been advanced through a number of cycles of operation the extreme end portion of the strip being shown in its ultimate form, that is with the walls of the corrugations bent for the purpose of closing or substantially closing the corrugations to form passageways. The pilot die 9 is for the purpose of piloting and guiding the stock, that is at each cycle it enters the adjacent corrugation of the strip and positions the strip properly.

When the machine is being operated at low speed, say 180 strokes per minute, the strip delivered to the machine, and from which the rings are formed, is of low carbon steel containing approximately 0.40 per cent to 0.50 per cent carbon. The preferred content of the steel utilized for low speed may be as follows:

|            | Per cent       |
|------------|----------------|
| Carbon     | 0.40 to 0.50   |
| Manganese  | 0.55 to 0.65   |
| Phosphorus | 0.009 to 0.011 |
| Sulphur    | 0.020 to 0.030 |
| Silicon    | 0.175 to 0.200 |

Low carbon steel provides an excellent material for the rings since the operations of swaging the metal give the material the desirable charac-

teristics of hard steel. If steel of the foregoing content were run through the machine at high speed, the result would be that fins would be formed at the sharp corners of the corrugations, since the soft metal would be forced between the dies into the working clearances by the impact.

In order to prevent flow of metal into the clearances of the slides or dies when the machine is operating at high speed, and for the purpose of efficiently swaging the sharp corners of the corrugation at high speed, a steel strip of higher carbon content is used. The steel for high speed production may have a content within the following ranges:

|            | Per cent       |
|------------|----------------|
| Carbon     | 0.70 to 0.75   |
| Manganese  | 0.48 to 0.50   |
| Phosphorus | 0.006 to 0.007 |
| Sulphur    | 0.031 to 0.032 |
| Silicon    | 0.130 to 0.135 |

By using a steel having 0.70 to 0.75 per cent carbon, the machine can be run at a speed of approximately 300 strokes per minute, without causing the formation of fins at the corners as heretofore described, since this metal of greater hardness will not flow into the clearances.

Having described my invention, I claim:

1. The method of fabricating a piston ring from a strip of metal consisting of the steps of, clamping the metal between opposing dies, bending the metal over the side of one of said opposing dies by means of a bending die and forming the crown of the corrugation between said bending die and an opposing die, bending the metal over the side of said bending die to form the other side wall of the corrugation and clamping the metal between another set of dies in alignment with the first set, thereafter retracting the bending die a slight amount and pressing the crown wall of the corrugation against said bending die by means of said die opposing said bending die, said opposing die having sharp corners whereby the corrugation is provided with sharp edges.

2. The method of forming a piston ring from a strip of metal comprising the steps of, forming a corrugation, supporting the side walls of the corrugation against displacement, engaging the crown wall of the corrugation between dies, one of which includes sharp corners for the purpose of swaging the crown wall, and forming a sharp crown thereon, retracting the other of said dies sufficiently to provide a swaging space, and thereafter moving said first die toward the retracted die and swaging the metal of the crown of the corrugation within the swaging space thus provided whereby the metal fills the sharp corners afforded between the supports for the side walls of the corrugation and the crown engaging surface of the lower die.

3. The method of fabricating a piston ring from a strip of metal consisting of the steps of, clamping the metal between opposing dies, bending the metal by means of opposing dies to form corrugations, thereafter retracting one of the dies engaging the crown of the corrugation sufficiently to provide a swaging space, and pressing the crown wall of the corrugation against said die within said space by means of the opposite die having sharp corners, whereby the corrugation is swaged to provide sharp edges.

VICTOR F. ZAHODIAKIN.